

Patented Dec. 5, 1939

2,182,081

## UNITED STATES PATENT OFFICE

2,182,081

## WOOD-TREATING COMPOSITION

Ira Hatfield, Webster Groves, Mo., assignor to  
 Monsanto Chemical Company, St. Louis, Mo., a  
 corporation of Delaware

No Drawing. Application May 10, 1938,  
 Serial No. 272,784

8 Claims. (CL 134—78.8)

The present invention relates to a process of preserving wood and similar cellulosic materials subject to attack by stain, decay and mold fungi, as well as other micro-organisms, and termites and other insect pests, and refers particularly to a composition for this purpose.

Pentachlorophenol, tetrachlorophenols and, to a lesser extent, lower polychlorophenols have been found to be especially useful toxic substances for the treatment of wood and wood products to preserve them from attack by molds and micro-organisms such as are responsible for staining and decay. For finished mill work, tetrachlorophenols and pentachlorophenol have been applied to the wood in the form of a liquid composition by dipping. One of the principal requirements of the solvent or carrier which was to be used in such coating or impregnating compositions was that it be readily volatile. Solvents which were used included pine oil, kerosene, Stoddard solvent naphtha, alcohols, etc. It was also essential that the liquid composition should penetrate and spread in the wood when dipped therein. For this purpose various liquids called penetrants have been added to facilitate penetration of the end grain of the wood, and other materials called spreaders, have been added to aid spreading in the wood at right angles to the grain.

However, considerable difficulty has been encountered in using liquid tetrachlorophenol and pentachlorophenol compositions containing volatile solvents such as solvent naphtha, pine oil, alcohols, etc., for wood coating and impregnation, since, as the solvents volatilize, the polychlorophenols creep or work to the surface of the wood and so-called "blooming" or crystallization occurs. The crystalline deposit which thus forms as a bloom on the surface, besides having an objectionable appearance on the wood, is easily disengaged by rubbing, brushing or even blowing. When blooming occurs, as it invariably does with such compositions containing volatile solvents, the full value of the treatment is thus not afforded. Besides representing a loss of toxic material when the crystals come to the surface of the wood, disengaged crystals from the wood surface may present a health hazard.

The principal object of the present invention is to provide a liquid wood-preserving composition containing polychlorophenols which will not bloom on wood or similar materials coated or impregnated therewith, and will thus reduce the health hazard and increase the efficacy of a treatment with polychlorophenols. It is a fur-

ther object of the invention to provide an improved liquid composition for this purpose and a method for its application which will produce deeper penetration of the wood and thus provide better protection against stain, decay and similar attacks by micro-organisms.

In my co-pending application, Serial No. 181,989, filed on December 27, 1937, of which this application is a continuation-in-part, I have disclosed that the above objects are admirably realized by using a liquid composition comprising rosin or a similar resinous substance, toxic agents such as polychlorophenols, for example, tetrachlorophenols or pentachlorophenol, and a solvent such as a high-boiling, relatively non-volatile oil such as petroleum fuel oil or similar material. An example of such a liquid wood-preserving composition is one consisting of 5 parts of rosin and 5 parts of pentachlorophenol dissolved in 90 parts of Shell Petroleum Corporation's No. 2 Mid-Continent fuel oil. Such compositions are applied to the wood either by dipping, spraying or brushing, and the solvent instead of evaporating rapidly, partially remains on the surface of the wood for a short period and gradually penetrates into the wood. The composition acts both as a penetrant and spreader in the body of the wood.

Heretofore in using liquid wood-preserving compositions containing volatile solvents, brushing or spraying were poor methods of applying the compositions because sufficient penetration could not be achieved. It was thus necessary to use dipping treatments in which the wood was subjected to contact with liquid compositions for periods differing according to the degree of penetration desired, which period might vary from several minutes to a matter of hours. These dipping treatments were in reality soaking treatments. By using the coating compositions disclosed in my co-pending application and in the present application the coating composition may be spread on the wood by brushing, spraying or dipping. Of course, dipping treatments are still a preferred method. The composition slowly penetrates into the coated wood as the surface becomes dry. The full penetration and distribution of the treating solution continues over a period of from several hours to a day or more, even after the oily film has disappeared from the wood surface. The penetration of the wood by the liquid composition even in a brush or spraying treatment is deeper than that obtained by soaking in heretofore used volatile liquid compositions for periods usually permitted in such

dipping treatments. Greater quantities of wood can therefore be treated by dipping in any particular dipping vat in a given period according to the invention, since the effectiveness of the treatment is not dependent solely upon the period the wood remains submerged in the treating solution. The solution continues to penetrate into the wood after the wood is removed from the liquid. Since the solvents used in the improved compositions possess high flash points the fire hazard is considerably reduced. The composition is also suitable for application to wood by pressure treatments according to the methods known in the art.

The rosin or similar resinous substance in the composition has several functions. Liquid compositions without rosin when made with high-boiling oils, for example, Shell No. 2 fuel oil or Standard Oil Company of Indiana Engine Distillate (Fuel Oil No. 1) still produce blooming on the surface of the wood, although a slight reduction in tendency is noted with various oils of this character. However, I have discovered, as disclosed in my co-pending application, that rosin and similar resinous substances added in suitable proportions completely suppress blooming. Furthermore, the rosin has an additional function in solubilizing the toxic phenol, for example, pentachlorophenol and tetrachlorophenols. Compositions thus prepared have a shorter drying time on the wood, that is, the surface of wood treated therewith is drier in a shorter period of time than that treated with a similar composition not containing a resin, and the period required for penetration of the composition throughout the wood is not lengthened. Wood treated with the composition of my invention shows just as deep penetration as that treated by means of compositions not containing a resin, and since my invention also contemplates the use of particular solvents which have both a spreading and a penetrating action, wood thus treated exhibits deeper penetration than that resulting from treatment with compositions prepared with volatile solvents or compositions containing volatile solvents together with so-called spreaders and penetrants.

With the compositions of the present invention, the paintability and puttability of the wood is not substantially impaired after treatment. Since the compositions dry rapidly when applied to a wood surface, the wood is ready for the application of putty and for painting shortly after treatment, and since the surfaces are dry and free from bloom rather than oily and coated with crystals, putty and paint adhere firmly thereto.

In producing the liquid coating and impregnating compositions I dissolve approximately 5% by weight of a tetrachlorophenol or technical mixtures of tetrachlorophenols, or pentachlorophenol in 90% by weight of a fuel oil or a similar petroleum hydrocarbon oil, preferably one having a high flash point. Smaller proportions of the polychlorophenol component may be used but the resulting impregnated wood is not as completely protected. Greater proportions of the toxic materials in the liquid compositions may be used but these greater additions are, of course, limited to some extent by the solvent power of the petroleum oil and by economic considerations. The compositions must be stable and must completely retain all the polychlorophenol without any separation or crystallization at outdoor temperatures. For prolonged fungicidal protection a wood impregnated with a composition containing 5% of polychlorophenol according to the method of the invention is eminently satisfactory.

The petroleum oils which I prefer for the purposes of the invention are those having characteristics within the approximate ranges given hereinbelow:

|                                                     |                    |    |
|-----------------------------------------------------|--------------------|----|
| Gravity A. P. I. at 60° F.                          | 20-40              | 10 |
| Flash point A. S. T. M. (Tag-<br>llabue Closed Cup) | 140° F. and higher |    |
| Viscosity Saybolt Universal<br>at 100° F.           | 30-40              |    |
| A. S. T. M. distillation range                      | 300°-750° F.       | 15 |

Petroleum solvents boiling at lower ranges than those hereinabove specified may be used provided they dissolve the desired proportion of the toxic chemical. The odor and color of the oil must also be considered for the particular application. For some purposes, odorous oils or oils of dark color are not objectionable but for certain uses where color must not be imparted to the wood, light-colored relatively odorless oils are essential. Oils of high boiling range are desirable, as hereinbefore stated.

Although petroleum oil solvents are specifically contemplated, high-boiling chlorinated solvents and aliphatic as well as aromatic solvents may be used. The rosin or similar resinous material has proven effective in preventing the "blooming" tendency which the solvents might engender. Of course, economic considerations are in favor of the use of petroleum solvents or their mixtures with small proportions of other solvents.

In using the compositions of the invention, different solvent mixtures may be used in the treatment of wood products of different thicknesses. Thus, for example, a mixture of low-boiling and high-boiling petroleum solvents is 40 eminently suitable for the preparation of compositions for treatment of thin wood boards. For thicker boards, greater proportions of high-boiling solvents are desirable to facilitate deeper penetration.

In my co-pending application referred to hereinabove I have specifically disclosed as resinous constituents of my improved wood-treating compositions, rosin, cumarone-indene resins, petroleum resins such as those sold under the trade name "Santo-Resin", rosin residues, ester gum, rosin esters, petroleum tar resins and resins derived from rosin such as that designated by the trade name "Vinsol".

Of the various resins found useful, ester gum and rosin esters similar thereto are considerably more effective in preventing blooming, and wood-treating compositions prepared therefrom possess a number of other unexpected advantages.

Ester gum is the product resulting from the esterification of rosin with glycerol and consists essentially therefore of glycerol abietate. Esters of rosin or abietic acid with other alcohols, monohydric as well as polyhydric, may be substituted therefor without substantial loss of the advantages resulting from the use of ester gum in my wood-treating compositions. The rosin esters are preferably neutral, that is, substantially completely esterified products. Rosin salts such as limed rosin are not the equivalent of rosin esters. Limed rosin forms some calcium pentachlorophenate in pentachlorophenol solutions and the calcium pentachlorophenate is more subject to leaching by water than pentachlorophenol.

In comparison with polychlorophenol wood-

treating compositions prepared with resin, those prepared with resin esters such as ester gum have lower solution temperatures, have a color which is more stable in the presence of metals 5 and somewhat smaller proportions of resin ester may be used to prevent blooming on wood, that is, ester gum, for example, is a somewhat more effective bloom-controlling constituent than resin.

10 Solution temperature is the lowest temperature at which a definite quantity of the polychlorophenol will dissolve completely in a definite quantity of solvent containing the resin which was previously dissolved therein. This temperature is determined by slowly heating the solvent containing the resin in which is suspended the polychlorophenol. The solubilizing effect of the resin is thereby compared with that of other resins by means of this determination.

15 The differences between compositions containing resin from those containing resin esters is illustrated in the following results:

Solution temperature.—Five grams of pure pentachlorophenol were added to 95 grams of 25 Shell No. 2 fuel oil. The mixture was heated slowly and stirred. The pentachlorophenol was dissolved completely when the temperature reached 44.5° C. By adding 5 grams of Grade-K resin to 90 grams of the same fuel 30 oil and after solution of the resin therein, adding 5 parts of pure pentachlorophenol and heating slowly as before, it was found that the solution temperature was 42.0° C., that is, the solution temperature was reduced to 2.5° C. as a result of 35 the presence of the resin. By using 5 grams of Synthe-Copal ester gum (Reichhold Chemicals) instead of the resin, the solution temperature was found to be 39.5° C. or a reduction of 5.0° C.

Color stability in presence of metals.—Compositions were prepared consisting of 5 parts by weight of pentachlorophenol, 90 parts by weight of Shell No. 2 fuel oil and 5 parts by weight of the resins indicated below. Each of these compositions were placed in black iron drums (I. C. C. 45 5 E) and their colors were observed at various intervals. The color was determined by comparison with NPA color standards. The following results were obtained:

Hydrogenated wood rosin—(Stabylite)—original 50 3 which darkened to 8+ in 16 hours

Grade-K—rosin—original 4 which darkened to 3 in 3 days

Paramet Pale Ester Gum No. 2—original 3½ which darkened to 8 in 3 months

55 Synthe-Copal Ester Gum—original 3 which darkened to 8 in 3 months and remained 8 for 3 additional months

The proportions of materials to be used in 60 preparing compositions of the invention may be varied. The possible variation will be limited by the solubility of the particular toxic substance in the particular solvent. The ratio of resin ester to toxic substance necessary to suppress blooming of the toxic substance in the 65 particular solvent and to provide compositions of desirable surface-drying time will also be variable but will generally be approximately equal to or greater than the weight of the 70 toxic substance. In general the toxic polychlorophenol should be present in proportions of from 2 to 5 or more parts by weight to 100 parts by weight of the composition. Greater than 5 parts by weight of polychlorophenol to 100 75 parts of the composition may be used if a solvent

having sufficient solvent power for the polychlorophenol is employed or if sufficient resin is used to increase the solvent power of the solvent for the polychlorophenol to the desired extent. The proportion of ester gum or similar resin ester for use in the compositions will vary from about 1 to 10 or more parts per 100 parts by weight of the composition depending upon the proportion of polychlorophenol present the blooming of which is to be prevented. Slight 10 differences in blooming of the compositions is noted with different woods and these variations may be considered in providing a composition for the particular use.

The liquid compositions of the invention are 15 applicable to the treatment of wood and wood products which are particularly subject to decay and stain, especially those materials which are subjected to humid and moist conditions which favor the development of stain and decay. They 20 are also useful for protecting these materials from termite attack. Cellulosic materials such as cloths, papers, wall boards and the like which are also subject to attack by micro-organisms and insects can be similarly treated with these 25 compositions.

The compositions may be modified by the addition thereto of secondary materials such as wetting agents, water-repellents, insect-repellents, fire retardants, pigments or dyes, substances 30 which exert a synergistic action on the chlorinated phenols and other materials having favorable action on the impregnation or penetration of the composition or have a desirable action in further protecting or enhancing the value of the 35 treated article.

In this specification and in the claims tetrachlorophenol is to be understood to signify any of the isomers or a mixture of the isomers. It is also to be understood that the foregoing description is but a preferred embodiment of the 40 invention and that changes and modifications may be made therein without departing substantially from the invention which is defined in the appended claims.

45 Although the foregoing description has been specifically directed to the use of tetrachlorophenols and pentachlorophenol as the toxic component of the composition it is evident that the blooming of compositions containing other chlorinated phenolic toxics such as chlorinated creosols, chlorinated coal tar acids, chlorinated wood-tar acids, chlorinated naphthols, and chlorinated hydroxydiphenyls may likewise be prevented.

50 What I claim is:

1. A non-blooming liquid coating and impregnating composition for the treatment of wood and similar cellulosic materials to protect them from decay by molds and micro-organisms, comprising a chlorinated phenol dissolved in a solvent therefor in sufficient concentration to provide, when applied to wood and cellulosic materials, substantial protection from attack and decay by molds and micro-organisms and having a 55 resin ester dissolved in said solvent in sufficient concentration to prevent blooming on wood and similar cellulosic materials treated with the liquid composition.

2. A composition as defined in claim 1 and further characterized in that the resin ester is an ester gum.

3. A composition as defined in claim 1 and further characterized in that the solvent is a petroleum solvent.

4. A composition as defined in claim 1 and further characterized in that the solvent is a petroleum hydrocarbon fuel oil having a boiling range within the range of approximately 300° to 750° F.
5. A composition as defined in claim 1 and further characterized in that the chlorinated phenol is a polychlorophenol selected from the group consisting of tetrachlorophenols and pentachlorophenol.
10. 6. A non-blooming liquid coating and impregnating composition for the treatment of wood and similar cellulosic materials to protect them from attack and decay by molds and micro-organisms, comprising a chlorinated phenol selected from the group consisting of tetrachlorophenols and pentachlorophenol dissolved in a petroleum hydrocarbon oil having a boiling range within the range of approximately 300° to 750° F. in sufficient concentration to provide, when applied to wood and similar cellulosic materials, substantial protection from attack and decay by molds and micro-organisms, and having ester-gum dissolved in said petroleum hydrocarbon oil in sufficient concentration to prevent bloom-
- ing on wood and similar cellulosic materials treated with the liquid composition.
7. A non-blooming liquid coating and impregnating composition for the treatment of wood and similar cellulosic materials to protect them from attack by molds and micro-organisms, comprising the following materials in approximately the following proportions: 5 parts by weight of pentachlorophenol, 5 parts by weight of ester gum, and 90 parts by weight of a petroleum hydrocarbon fuel oil having a boiling range within the range of approximately 300° to 750° F.
8. A non-blooming liquid coating and impregnating composition for the treatment of wood and similar cellulosic materials to protect them from attack by molds and micro-organisms and insects, comprising the following materials in approximately the following proportions: 5 parts by weight of tetra-chlorophenol, 5 parts by weight of ester gum, and 90 parts by weight of a petroleum hydrocarbon fuel oil having a boiling range within the range of approximately 300° to 750° F.

15 20  
20  
20  
IRA HATFIELD.